

## UNITED STATES PATENT OFFICE

2,018,490

METHOD OF PRODUCING PAPER PULP  
FROM FIBROUS MATERIAL

Edwin P. Jones, Garden City, and James M. Dempsey, New York, N. Y., assignors to Cham-pagne Paper Corporation, New York, N. Y., a corporation of New York

No Drawing. Application April 10, 1935,  
Serial No. 15,620

8 Claims. (Cl. 92—11)

Our present invention relates to the manufacture of paper, and the like from cellulose containing materials, and more particularly to an improved method of preparing pulp to be used in such manufacture.

Specifically, our present invention relates to an improved method of producing a satisfactory pulp for paper making from crude decorticated bast fiber, such as flax or hemp, which either has or has not been first subjected to the usual and ordinary retting process.

An object of our invention is an improved method of producing a better quality of paper pulp from decorticated flax or hemp than has been heretofore possible.

Another object of our invention is an improved method of treating fibrous material, derived from flax or hemp stalks, to produce a pulp having strength, color, and other characteristics superior to that produced by previously known methods.

In the previously known methods of producing paper pulp from fibrous material, derived from flax or hemp stalks, it is the practice to subject the fibrous material to a chemical treatment for the purpose of loosening and removing, to a more or less degree, the lignins and incrustants which bind the fibers together, so that the fibers may be easily separated. After such chemical treatment the separated fibers, are ordinarily subjected to a bleaching process to increase the whiteness of the fibers to the desired degree.

Because of the limitations imposed on this bleaching process, it has been necessary to sacrifice, to some degree, the quality of the finished pulp. This has been true with respect to certain types of fibrous material, particularly flax, in which a very large proportion of the fibrous material must be destroyed during processing, if the hard fiber bundles or shives are sufficiently treated to permit of securing a resulting final pulp of satisfactory whiteness with known bleaching methods.

In our present invention we have departed radically from heretofore known methods of producing paper pulp from fibrous materials such as flax or hemp.

Mechanically decorticated flax which is suitable as a raw material should contain approximately 90% crude bast fiber and the remainder of the shives and other impurities. The shives are in reality a mixture of the inside of the flax stalk and a small percentage of the outside, or bark, of the plant. We have ascertained that the mechanically decorticated flax contains between

10% and 20% of water-soluble substances, and as a first step in my improved process we steep the flax for a short period of time in water. Such period of time may vary from fifteen to 30 minutes.

We find that it is quite immaterial whether hot or cold water is employed, as the water-soluble substances are dissolved with equal facility in either. Cold water is employed however, and we find that the same dissolves these water-soluble substances in a satisfactorily short period of time.

We find further that we can facilitate the subsequent steps of our improved method or process by allowing the above referred to steeping in water to take place while the fibrous material is being subjected to the action of a beater, a rod mill, or similar equipment. Therefore, in practice, the first step in our improved process consists in passing the mixture of mechanically decorticated flax through a continuously operated equipment (such as beaters, rod mills, etc.) which imparts a crushing, rather than a cutting action to the raw material.

After the fibrous material has been treated as above described, it is thoroughly washed to remove the dissolved matter. The fibrous material is then placed in a rotary digester, where it is cooked at an appropriate temperature and pressure for a predetermined length of time. The time, temperature, and pressure will vary according to the character of the material being worked upon, but we have obtained satisfactory results by cooking the material under a pressure of approximately 50 pounds per square inch for a period of approximately two hours. However, we are of the opinion that the concentration and combination of chemicals employed in this digesting step are of more importance than either the temperature, pressure or length of time of cooking.

We have found that a cooking reagent composed of practically any alkaline chemical in combination with a soluble sulphite will give satisfactorily digested material. I prefer however, a mixture of approximately 95% of either calcium hydroxide, sodium carbonate or sodium hydroxide with about 5% sodium sulphite. Also, we may employ a mixture of two or more of the above stated materials in approximately equal proportions in combination with sodium sulphite, the mixture constituting approximately 95% of the combination. The proportions of the alkaline chemicals employed, to the dry weight of the decorticated fiber, may vary from 5-15%. The actual concentration of the chemicals expressed

as pounds of total chemicals in relation to the total number of pounds of water present in the cooking medium is not critically important, but is dependent rather upon the shape of the digester employed. After the digester is blown, the cooked fiber is thoroughly washed in water to remove the dissolved material.

An inspection of the digested fiber shows that the bast fiber itself has been materially whitened, whereas the shives have taken on a decided brownish cast. An inspection of the shives discloses that they have lost a large part of their strength and have become much softer.

The next, and equally important, part of our improved process or method comprises bleaching the shives without at the same time sacrificing the strength of the bast fiber itself. It is practically impossible to bleach the cooked conglomerate (that is, bast fiber and shives), using an alkaline hypochlorite in a single stage bleach, so as to produce a satisfactory pulp. Therefore, we have utilized as this part of the invention what may be termed a two-stage bleach.

In the first stage bleach the digested conglomerate is treated with a predetermined quantity of either saturated chlorine water or hypochlorous acid or gaseous chlorine. It is ordinarily necessary to use approximately 2-3 grams of chlorine for each 100 grams of conglomerate. The amount actually used must of necessity depend upon both the quantity of shives present in the conglomerate, as well as the thoroughness of the previously described digestion. The shives absorb or react with either the chlorine water, gaseous chlorine or hypochlorous acid, immediately upon exposure to the chemicals mentioned.

In any event, the bast fiber is lightened in color immediately and the shives turn a deep brownish-red color, indicating that the chlorine reacts very quickly upon both the bast fiber and the shives. At the end of about 15 to 30 minutes, depending upon whether or not agitation of the mixture is employed, practically all of the available chlorine has been consumed.

The mixture is now washed, either with water or with a mild solution of any of the common alkalies, such as sodium hydroxide, sodium carbonate, or the like.

The material is now ready for the second stage of the two-stage bleaching process, which consists in treatment with an alkaline hypochlorite.

The mixture of reddish brown shives and comparatively white bast fiber is placed in a solution of either sodium or calcium hypochlorite. The former appears to work better than the common bleaching solution of calcium hypochlorite and is to be preferred thereto, although good results may be obtained with the latter.

The mixture is allowed to remain in the bleaching solution at room temperature for approximately seven hours, when it will be found that the heretofore small reddish-brown shives have become practically white, and can hardly be found in the mass of bast fibers which have now reached a satisfactory color.

To bring about satisfactory bleaching in this stage of the process, we find it advantageous to use the equivalent of approximately 2-4 pounds of ordinary bleaching powder per 100 pounds of conglomerate.

After this second step of the two-stage bleaching process, the pulp is thoroughly washed to remove all of the bleaching liquor, and the pulp is then ready to be used in subsequent steps in the making of a high quality paper.

The various steps of our process may be varied to suit different conditions, depending largely on the nature of the material being worked upon. The process may be practiced with the use of apparatus which will permit of the continuous treatment of the fibers from the decorticating step to the passing of the completely prepared pulp to the paper making machine.

We claim.

1. The improved method of producing paper 10 pulp from flax, which consists in submitting mechanically decorticated flax to the action of water, washing the same, cooking the fibers in a digester in the presence of an alkaline chemical in combination with a soluble sulphite and then 15 bleaching the fibers.

2. The improved method of producing paper pulp from decorticated flax which consists in steeping the same in water to dissolve soluble matter contained therein, washing the same to 20 remove the dissolved matter, cooking in a digester in the presence of an alkaline chemical in combination with a soluble sulphite, and then bleaching the same.

3. The improved method of producing paper 25 pulp from a conglomerate of bast fiber and shives, which consists in steeping the conglomerate in water, to dissolve the soluble matter contained therein, washing the conglomerate to remove the dissolved matter, cooking the conglomerate in a 30 digester in the presence of an alkaline chemical in combination with a soluble sulphite, washing the conglomerate, and then subjecting the conglomerate to a two-stage bleaching operation.

4. The improved method of producing paper 35 pulp from a conglomerate of bast fiber and shives, which consists in steeping the conglomerate, to dissolve soluble matter contained therein, washing the conglomerate to remove the dissolved matter, milling the conglomerate to crush and 40 soften the shives, cooking the conglomerate in a digester in the presence of an alkaline chemical in combination with a soluble sulphite, washing the conglomerate, treating the conglomerate with chlorine in the presence of water, washing the 45 conglomerate, and then treating the conglomerate with an alkaline hypochlorite.

5. The improved method of producing paper pulp from a conglomerate of bast fiber, shives, and soluble impurities, which consists in steeping the conglomerate, to dissolve the soluble impurities, washing the conglomerate to remove the dissolved impurities, milling the conglomerate to crush and soften the shives, cooking the conglomerate in a digester with a reagent composed of approximately 95% sodium carbonate and approximately 5% sodium sulphite, under pressure, washing the conglomerate, treating the conglomerate with a solution of chlorine, washing the conglomerate, then treating the conglomerate with a solution of sodium hypochlorite for approximately seven hours at room temperature, and then washing the conglomerate.

6. The improved method of producing paper pulp from a conglomerate of bast fiber, shives, 65 and soluble impurities, which consists in steeping the conglomerate, milling the conglomerate, cooking the conglomerate in a digester with a reagent composed of approximately 95% of sodium hydroxide and approximately 5% of sodium sulphite under a pressure of from 30-75 pounds per square inch, treating the conglomerate with chlorine in the presence of water, and treating the conglomerate with a common bleaching agent for approximately seven hours, the conglomerate 70

being thoroughly washed between each step of the method.

7. The improved method of producing paper pulp from a conglomerate of bast fiber and shives, which consists in steeping the conglomerate, to dissolve soluble matter contained therein, washing the conglomerate to remove the dissolved matter, cooking the conglomerate in a digester in the presence of an alkaline chemical in combination with a soluble sulphite, washing the conglomerate, milling the conglomerate to crush and soften the shives, treating the conglomerate with chlorine in the presence of water, washing the conglomerate, and then treating the conglomerate with an alkaline hypochlorite. 5

8. The improved method of producing paper pulp from a conglomerate of bast fiber, shives, and soluble impurities, which consists in steeping

the conglomerate, to dissolve the soluble impurities, washing the conglomerate to remove the dissolved impurities, milling the conglomerate to crush and soften the shives, cooking the conglomerate in a digester under pressure with a reagent composed of a mixture of calcium hydroxide, sodium carbonate and sodium hydroxide in combination with sodium sulphite, and with the mixture constituting approximately 95% of the combination, washing the conglomerate, treating 10 the conglomerate with a solution of chlorine, washing the conglomerate, then treating the conglomerate with a solution of sodium hypochlorite for approximately seven hours at room temperature, and then washing the conglomerate. 15

EDWIN P. JONES.  
JAMES M. DEMPSEY.